# EUROPEAN PATENT SPECIFICATION

(11) **EP 0 475 633 B1**
(45) Date of publication and mention of the grant of the patent: **15.02.1995**
(21) Application number: 91307857.2
(22) Date of filing: 28.08.1991
(51) Int. Cl.: B41M 5/00

(54) **Thermal transfer printing receiver sheet**
Bildempfangsmaterial für thermische Farbstoffübertragung
Matériau récepteur d'image pour le transfert thermique

(30) Priority: 14.09.1990 JP 245382/90
(43) Date of publication of application: 18.03.1992
(73) Proprietor: IMPERIAL CHEMICAL INDUSTRIES PLC, London SW1P 3JF (GB)
(72) Inventor: Kiyotaka, Sakata, Tsukuba-shi, Ibaraki-ken (JP); Kazuhiko, Iiyama, Tsukuba-shi, Ibaraki-ken (JP)
(74) Representative: Hall, David Brian

(56) References cited:
- EP-A- 0 464 921

## Description

This invention relates to thermal transfer receiver sheets which are used in combination with a thermal transfer dyesheet containing thermal transfer dyes and employing heating means (such as thermal heads) to transfer dye from the dyesheet to a dye-receiving layer on the receiver sheet, according to image signals applied to the heating means. The invention relates especially to an improved dye-receiving composition.

Thermal transfer printing systems have been developed in recent years for producing images by causing thermal transfer dyes to transfer to a receiver sheet in response to thermal stimuli. Using a dyesheet comprising a thin substrate supporting a dyecoat containing one or more such dyes uniformly spread over an entire printing area of the dyesheet, printing is effected by heating selected discrete areas of the dyesheet while the dyecoat is pressed against a dye-receptive surface of a receiver sheet, thereby causing dye to transfer to corresponding areas of the receiver. The shape of the image thus formed on the receiver is determined by the number and location of the discrete areas which are subjected to heating.

High resolution photograph-like prints can be produced by thermal transfer printing using appropriate printing equipment, such as programmable thermal heads or laser printer, controlled by electronic image signals derived from a video, computer, electronic still camera, or similar signal generating apparatus. Thus for example a thermal print head has a row of individually operable tiny heaters spaced to print typically six or more pixels per millimetre. Selection and operation of these heaters is effected according to the electronic image signals fed to the printer.

Full colour prints can be produced by printing with different coloured dyecoats sequentially in like manner, and the different coloured dyecoats are usually provided as discrete uniform print-size areas in a repeated sequence along the same dyesheet.

Receiver sheets comprise a substrate sheet supporting a dye-receiving layer containing a material having an affinity for the thermal transfer dye molecules, and into which they can readily diffuse when an adjacent area of dyesheet is heated during printing. Such materials are mainly constituted by various aromatic or aliphatic polyesters, as described for example in JP-A-57-107,885, JP-A-61-258,790, JP-A-1-269,589 and US 4,474,859. Layer compositions comprising copolyesters of 1,4-cyclohexanedicarboxylic acid and 1,4-cyclohexane dimethanol have been disclosed in EP-A-0 464 921 which constitutes prior art according to Art. 54(3) EPC. A thermal transfer printing receiver sheet comprising a dye-receiving layer is, however, not disclosed therein.

When previously known aromatic and aliphatic polyesters were used for the dye-receiving layer of the receiver sheet, one or more of a number of problems were usually experienced. Thus with some polyesters, the maximum optical densities that could be obtained under normal printing conditions, were insufficient, due to inferior dye-receiving properties of the polyester used. Other problems that were often experienced included poor stability of the image, giving deterioration of the image during storage, a fault which can be accelerated for measuring by exposing the printed sheet to high temperature and high humidity conditions. Light fastness of the printed image, and resistance to the development of finger prints, are also desirable properties that are influenced by the material selected for the dye-receiving surface. We have now devised a new receiver sheet having an improved balance of such properties.

According to the present invention, a thermal transfer printing receiver sheet comprises a substrate supporting a dye-receiving layer on its surface, characterised in that the vain constituent of the dye-receiving layer is a copolyester in which the acid component comprises at least one alicyclic dicarboxylic acid, and the alcohol component comprises at least one alicyclic diol.

Materials suitable for use as the substrate of the receiver sheet may variously include for example, thermoplastic films, synthetic papers and cellulose fibre papers. Examples include films or sheets of polyester, polyvinyl chloride, polypropylene, polyethylene. polycarbonate, polyimide, polyamide, polyamideimide, especially biaxially orientated polyethyleneterephthalate film. Examples of synthetic papers include those of fabricated and moulded polyolefines, polystyrene, and polyesters etc. as the polymer component. Cellulose fibre papers, woodfree paper, coated paper, art paper, synthetic rubber latex impregnated paper, cast-coated paper, etc, can also be used. The above may be used on their own, although a laminated substrate using a combination of two or more of the above, may be preferred for some applications.

The substrate supports the dye-receiving layer, which is provided as a coating on its surface for the purpose of receiving the dyes transferred from selected areas of the dyesheet, thereby to form an image. The main constituent of the dye-receiving layer of the present invention is a copolyester formed by using an acid component comprising at least one alicyclic dicarboxylic acid.

Examples of alicyclic dicarboxylic acids which can be used for this purpose, include cyclopropane dicarboxylic acid, cyclobutane dicarboxylic acid, cyclohexane-1,2-dicarboxylic acid, cyclohexane-1,3-dicarboxylic acid, cyclohexane-1,4-dicarboxylic acid, methylhexahydrophthalic acid, and norbornene dicarboxylic acid. In furtherance of this invention, the alicyclic acid components of the copolyester can be introduced as the acid or as the corresponding anhydride, as appropriate. Examples of such anhydrides, for example, include hexahydrophthalic acid anhydride, and methyl-hexahydrophthalic acid anhydride.

The acid component of the copolyester may also include other polybasic carboxylic acids, such as those previously used on their own without the present alicyclic acids. Such other dicarboxylic acids may include, for example, aromatic dicarboxylic acids such as terephthalic acid, isophthalic acid, orthophthalic acid, 2,6-naphthalene dicarboxylic acid, etc, aliphatic dicarboxylic acids, such as succinic acid, adipic acid, azelaic acid, sebacic acid, dodecane dicarboxylic acid, etc. Tri- and tetra-carboxylic acids, such as trimellitic acid, trimesic acid, pyromellitic acid, etc, may also be added to the alicyclic dicarboxylic acid.

When the acid component of the copolyester comprises a mixture of alicyclic dicarboxylic acids and other polybasic carboxylic acids, we prefer the molar ratio of the alicyclic dicarboxylic acids to the other carboxylic acids in the mixture to be within the range 5/95 - 95/5, especially within the range 10/90 - 50/50, the range 10/90 - 30/70 being particularly preferred with some acid combinations.

The alcohol component of the copolyester of the present invention comprises at least one alicyclic diol. Examples of diols that can be used for this purpose include 1,4-cyclohexanedimethanol, cyclohexane-1,2-diol, cyclohexane-1,3-diol, cyclohexane-1,4-diol, cyclopentane-1,2-diol, cyclopentane-1,3-diol, tricyclodecanedimethylol, and ethylene oxide adduct of hydrogenated Bisphenol A.

The alcohol component of the copolyester may also include other polyols, such as those previously used on their own in the absence of the present alicyclic diols, for example. Such additional other polyols may include ethylene glycol, propylene glycol, butanediol, neopentyl glycol, diethylene glycol, 1,6-hexanediol, 2,2-diethyl-1,3-propanediol, 2-n-butyl-2-ethyl-1,3-propanediol, and ethylene oxide and/or propylene oxide adduct of Bisphenol A, and polyols such as trimethylol propane, glycerin, pentaerithritol, polyglycerin, etc.

When the alcohol component of the copolyester comprises a mixture of alicyclic diols and other polyhydric alcohols, we prefer the molar ratio of the alicyclic diols to the other alcohols in the mixture, to be within the range 5/95 - 95/5, especially within the range 10/90 - 50/50, the range 10/90 - 30/70 being particularly preferred with some polyol combinations.

Dye-receiving layers of the present invention can be made by coating a substrate with a composition containing the copolyester, using any of the normal coating techniques, such as roll coating or gravure printing, for example. The viscosity of the coating composition can be adjusted by altering the amount of solvents present, and these are subsequently removed from the applied layer by drying. Receivers made according to the invention, can show properties superior to those obtained with previously known polyesters, but such improvements are only shown when both alicyclic dicarboxylic acid and alicyclic diol moieties are present; ie not when only one or the other is present.

In order to improve release from the thermal transfer dye-sheet after printing, the thermal printing receiver may be provided with a release agent in the dye-receiving layer or on its surface. Examples of release agents include solid waxes such as polyethylene wax, amide wax, polytetrafluoroethylene powder, fluorine- or phosphate-type surfactants, and especially silicone oils.

Both oil type and solid type silicone oils can be used, but curable silicone materials are preferred. Where such release system is to be used on the surface of the receiver, the uncured silicone materials are first applied as an uncured coating composition on the dye-receiving layer, dried as appropriate, and thereafter cured in situ. Where the release system is to be contained in the dye-receiving layer, the curable materials are mixed with the copolyester in a coating composition, which is then applied to the substrate and dried, curing of the release system then being effected in situ. Such cross-linked matrices these produce within the dye-receiving layer help to stabilise it. They can be reaction curing types, photocuring type or catalytic curing type, for example, but the reaction curing type is preferred.

Examples of reaction curing release systems include the reaction products of amino-modified silicone oils, such as KF-393, KF-857, KF-858, X-22-3680, X-22-3810 (these being products of Shin-Etsu Chemical), and M468 (ICI), reacted with an epoxy-modified silicone such as KF-100T, KF-101, KF-103 (these also being products of Shin-Etsu Chemical), or with an organic oligoepoxide free from silicone, such as Diepoxide 126, Diepoxide 183 (both being products of Degussa), and Araldite GY 1558 GB (Ciba Geigy). Preferred quantities of such release systems in the dye-receiving layer are 0.05-20% of the copolyester.

The cross-linking of the copolyester can also be enhanced, by including an effective amount of a cross-linking agent in the coating composition, applying this as a layer to the substrate, and carrying out the cross-linking reaction in situ, ie in essentially the same manner as that described above for the release system. Examples of crosslinking agents include compounds having isocyanate groups, compounds having active methylol or alkoxy methyl groups, acid anhydride, carboxy groups, or epoxy groups. It is generally preferred to limit the crosslinking agent to 0.5-20 wt % of the copolyester.

In addition to the copolyester of the present invention and any polymeric release agent that might be employed, the dye-receiving layer may also contain a minor amount of other polymeric materials intimately mixed with the copolyester. Examples of such other polymeric materials include polyvinyl chloride, polyvinyl acetate, vinyl chloride/vinyl acetate coplymer, polystyrene, polycarbonate, acrylic and methacrylic polymers, cellulosic polymers, polyacetal, polyethylene, and polypropylene; and even thermosetting resins such as epoxy, melamine, urethane and urea type resins can be present in small quantities. By minor amount, we mean less than 50 % by weight, and prefer there to be less than 20 % of the other polymer. For most purposes we particularly prefer that no such other polymer be included in the dye-receiving layer, any polymeric material in the dye-receiving layer being limited to the copolyester and any polymeric release agent.

The dye-receiving layer may also contain stabilisers for combating fading and/or a UV absorber. Suitable quantities are 0.5-20 wt % of the copolyester.

To obtain a smoother gradation of colour, especially when using a hard substrate, can be obtained by providing an intermediate compliant layer between the substrate and the dye-receiving layer. Such layers may be in the form of a compliant cushion or a porous layer, and these may be formed from polyurethane, polyester, polyamide, acrylic or methacrylic polymers, or synthetic rubber. The thickness of such layers may suitably be in the range 1-50 »m.

In order to control the formation of static electricity, during the fabrication process or while travelling through the printer with the dyesheet, an antistatic agent can be coated onto or incorporated with one or more coating of the receiver. We prefer that antistatic treatments be applied to both sides of the substrate.

### EXAMPLES

Evaluation of thermal printing receiver sheets according to the invention was made by transferring images onto the dye-receiving layer using a thermal head. The receiver sheet was placed against a dyesheet with its dye-receiving layer in contact with the dyecoat of the dyesheet (details of the latter being specified in the example below). Heat was applied to the back of the dyesheet by a thermal head having an output energy of 0.32 W/dot, a head heating time of 6 ms and a dot density of 6 dots/mm. The printed sheets thus formed were evaluated in respect of their optical density, light fastness, storage stability, and finger print resistance, in the following manner.

### Optical density

The image density was measured on a SAKURA optical density meter PDA 85.

### Light fastness

The hue of the image was measured before and after accelerated aging of the print by ATRAS HPUV, to determine the change in hue which occurred during the aging cycle.

### Storage stability

The printed receiver sheet was stored in an atmosphere of 45°C and 85% relative humidity, for 2 weeks. The hue was again measured before and after treatment, to determine the change of hue occurring under those conditions.

### Finger print resistance

The optical density of the printed image was determined. A finger print was then made on the image surface, and the print left in an atmosphere of 45°C and 85% relative humidity for 2 weeks. After that time the optical density was again measured of the part of the print on which the finger print had been made. The change in optical density was recorded as a percentage of the initial measurement.

### Production of copolyester (A)

245.6 parts of dimethyl terephthalic acid, 69.4 parts of ethylene glycol, 2.9 parts of trimethylol propane, 211.1 parts of 2-n-butyl-2-ethyl-1,3-propanediol, 118.5 parts of 1,4-cyclohexane dimethanol and 0.1 part of zinc acetate were placed into a flask installed with a thermometer, nitrogen gas inlet tube, reflux dehydrator and stirrer, and it was heated at 170°C - 220°C for 5 hours. During the heating, methanol formed was evaporated outside the system. Then it was cooled at 170°C, 105.1 parts of isophthalic acid and 97.5 parts of hexahydrophthalic anhydride were added and the mixture heated at 170°C - 230°C for 6 hours. During the heating, water formed was evaporated outside the system. The reflux dehydrator was then replaced with a vacuum pressure reducer, and after an addition of 0.1 part of antimony trioxide, it was heated at 260°C and 666 Pa (5 mmHg) pressure for 4 hours, to perform the reduced pressure condensation reaction from which the copolyester (A) was obtained.

The reactants used for the production of the copolyester (A) are summarised below.

### Example 1

### Preparation of thermal transfer receiver sheet

Receiver sheet (a′) was prepared by wire bar coating one surface of a polyester film with an ink composition (a), and drying this to produce a dye-receiving layer of approximately 5 »m thickness. The polyester film was Melinex 990 (Melinex is a trade mark of Imperial Chemical Industries PLC, hereinafter referred to as ICI). Ink composition (a) contained copolyester (A) as the main constituent of the dye-receiving layer, a release system also being present as a minor constituent. The full composition of ink composition (a), is set out below.

### Preparation of the thermal transfer dye sheet

A slipping layer of silicone oil was formed on one side of a 6 »m polyester substrate film (Lumilar Toray product). Then an ink composition (I) for the thermal transfer printing was prepared as described below, and was coated onto the other surface of the substrate from that coated with the slipping layer. The ink composition (I) was then dried to form a 1.0 »m thick dyecoat, to complete the thermal transfer dye sheet (I′). Details of the ink composition were as follows:

Then the thermal transfer dye sheet (I′) and the thermal transfer printing receiver sheet (a′) were held together, and an image was formed in the dye-receiving layer by heating with a thermal head. The optical density, light fastness, storage stability and finger print resistance of the printed sheet thus produced, were evaluated. The results are shown in Table I.

### Example 2

An ink composition (b) for forming a dye receiving layer was prepared in the similar manner to that in Example 1, but using copolyester (B) as the main constituent. A thermal transfer printing receiver sheet (b′) was prepared by coating this ink onto Melinex 990 and drying, as described above. Using the thermal transfer dyesheet (I′) to provide the transfer dyes, a printed sheet was obtained by forming an image in the dye-receiving layer of receiver sheet (b′), by heating with a thermal head. The optical density, light fastness, storage stability and finger print resistance were then evaluated. The results are shown in Table l.

### Example 3

An ink composition (c) was prepared in the similar manner to the two preceding Examples, but using copolyester (C) as the main constituent, and thermal transfer printing receiver sheet (c′) was prepared and printed in like manner. The optical density, light fastness, storaae stability and finger print resistance of the resultant print were then evaluated, and the results are shown in Table I

### COMPARATIVE EXAMPLES

Copolyester resins (D) and (E) were prepared from the compositions shown below, in similar manner to those of Examples 1 to 3 above.

| Copolyester (D) | |
|---|---|
| dimethyl phthalic acid | 187.0 parts |
| isophthalic acid | 240.0 parts |
| ethylene glycol | 77.0 parts |
| neopentyl glycol | 195.4 parts |

| Copolyester (E) | |
|---|---|
| dimethyl phthalic acid | 187 0 parts |
| isophthalic acid | 240.0 parts |
| trimellitic anhydride | 13.7 parts |
| ethylene glycol | 77.0 parts |
| neopentyl glycol | 195.4 parts |

### Comparative Example C1

An ink composition (d) for forming the dye-receiving layer was prepared in a similar manner to that of Example I but using copolyester (D) as the main constituent, and a corresponding thermal transfer printing receiver sheet (d′) was prepared, again using Melinex 990 as substrate. Thermal transfer dyesheet (I′) and thermal transfer printing receiver sheet (d′) were passed together through a thermal printer, and a printed sheet was obtained by forming an image in the receiver layer by heating with the thermal head. Optical density, light fastness, storage stability and finger print resistance of the printed sheet, were evaluated. The results are shown in Table 1.

### Comparative Example C2

An ink composition (e) for forming the dye receiving layer was prepared in similar manner to those of the preceding Examples, but using copolyester (E) as the main constituent. Receiver sheet (e′) was prepared by coating Melinex 990 with a layer of e. This was printed as before using thermal transfer dyesheet (I′) and the optical density, the light fastness, the storage stability and the finger printing resistance were evaluated. The results are shown in Table l.

**Table 1**

| | Example | | | Comparative Example | |
|---|---|---|---|---|---|
| | (1) | (2) | (3) | (C1) | (C2) |
| Optical Density | 1.2 | 1.3 | 1.2 | 1.0 | 0.9 |
| Light Features | 20.0 | 20.5 | 20.0 | 23.0 | 24.0 |
| Storage Stability | 2.0 | 3.0 | 2.5 | 6.0 | 7.0 |
| Finger Print Resistance (%) | +3.0 | +2.0 | +4.0 | -8.0 | -10.0 |

To summarise these observations, when general polyester resins as used previously, were used as the main constituent of the dye receiving layer, it was difficult to satisfy all the required properties of optical density, light fastness, storage stability and finger print resistance. However, by using copolyesters obtained by reacting at least one alicyclic dicarboxylic acid as the acid component for the copolymerization and at least one alicyclic diol as the alcohol component, these properties can be largely improved. Such receivers enable a printed sheet with an image of high quality, having a superior balance of properties with respect to optical density, light fastness, storage stability and finger print resistance, to be obtained.

## Claims

1. A thermal transfer printing receiver sheet comprising a substrate supporting a dye-receiving layer on its surface, wherein the main constituent of the dye-receiving layer is a copolyester in which the acid component comprises at least one alicyclic dicarboxylic acid, and the alcohol component comprises at least one alicyclic diol.

2. A thermal transfer printing receiver sheet as claimed in claim 1, wherein the acid component of the copolyester comprises a mixture of an alicyclic dicarboxylic acid component and an other polycarboxylic acid component, having a molar ratio within the range 5/95 - 95/5.

3. A thermal transfer printing receiver sheet as claimed in claim 2, wherein the acid component of the copolyester comprises an alicyclic dicarboxylic acid component and an aromatic dicarboxylic acid component.

4. A thermal transfer printing receiver sheet as claimed in claim 3, wherein the aromatic dicarboxylic acid component is present in a greater molar proportion than the alicyclic dicarboxylic acid component.

5. A thermal transfer printing receiver sheet as claimed in claim 3 or claim 4, wherein the aromatic dibasic acid component comprises at least one terephthalic acid or isophthalic acid.

6. A thermal transfer printing receiver sheet as claimed in claim 1, wherein the alcohol component of the copolyester comprises a mixture of an alicyclic diol component and an other polyhydric alcohol component, having a molar ratio within the range 5/95 - 95/5.

7. A thermal transfer printing receiver sheet as claimed in claim 6, wherein the alcohol component of the copolyester comprises an alicyclic diol component and an aromatic diol component.

8. A thermal transfer printing receiver sheet as claimed in claim 7, wherein the aromatic diol component is present in a greater molar proportion than the alicyclic diol component.

9. A thermal transfer printing receiver sheet as claimed in claim 8, wherein the aromatic component of the diol mixture comprises an ethylene oxide or propylene oxide adduct of a bisphenol.

10. A thermal transfer printing receiver sheet as claimed in claim 1, wherein the alicyclic diol component of the polyester has a cyclohexane skeleton.

11. A thermal transfer printing receiver sheet as claimed in any one of the preceding claims, wherein in addition to the copolyester and any polymeric release agent that might he employed, the dye-receiving layer contains a minor amount of other polymeric materials intimately mixed with the copolyester.

12. A thermal transfer printing receiver sheet as claimed in any one of the preceding claims, wherein the polyester-type cross-linking of the copolyester is enhanced by reaction with an effective amount of a cross-linking agent therefor.

13. A thermal transfer printing receiver sheet as claimed in any one of the preceding claims, in which an antistatic agent is coated onto or is incorporated within one or more coatings of the receiver.

14. A thermal transfer printing receiver sheet as claimed in claim 13, wherein the antistatic treatments are applied to both sides of the substrate.

15. A thermal transfer printing system comprising a dyesheet containing thermal transfer dyes and a receiver sheet for receiving the dyes during thermal transfer printing, wherein said receiver sheet is a receiver sheet as claimed in any one of claims 1 to 14.

## Patentansprüche

1. Empfangsblatt für den Thermotransferdruck, umfassend einen Träger, der auf seiner Oberfläche eine farbstoffempfangende Schicht stützt, wobei der Hauptbestandteil der farbstoffempfangenden Schicht ein Copolyester ist, in dem die saure Komponente wenigstens eine alicyclische Dicarbonsäure umfaßt und die Alkoholkomponente wenigstens ein alicyclische Diol umfaßt.

2. Empfangsblatt für den Thermotransferdruck nach Anspruch 1, worin die saure Komponente des Copolyesters eine Mischung aus einer alicyclischen Dicarbonsäurekomponente und einer anderen Polycarbonsäurekomponente umfaßt, die ein molares Verhältnis im Bereich von 5:95 bis 95:5 aufweisen.

3. Empfangsblatt für den Thermotransferdruck nach Anspruch 2, worin die saure Komponente des Copolyesters eine alicyclische Dicarbonsäurekomponente und eine aromatische Dicarbonsäurekomponente umfaßt.

4. Empfangsblatt für den Thermotransferdruck nach Anspruch 3, worin die aromatische Dicarbonsäurekomponente in einem größeren molaren Anteil als die alicyclische Dicarbonsäurekomponente anwesend ist.

5. Empfangsblatt für den Thermotransferdruck nach einem der Ansprüche 3 oder 4, worin die aromatische dibasische Säurekomponente wenigstens eine der beiden folgenden Säuren umfaßt: Terephthalsäure oder Isophthalsäure.

6. Empfangsblatt für den Thermotransferdruck nach Anspruch 1, worin die Alkoholkomponente des Copolyesters eine Mischung aus einer alicyclischen Diolkomponente und einer anderen mehrwertigen Alkoholkomponente umfaßt, die ein molares Verhältnis im Bereich von 5:95 bis 95:5 aufweisen.

7. Empfangsblatt für den Thermotransferdruck nach Anspruch 6, worin die Alkoholkomponente des Copolyesters eine alicyclische Diolkomponente und eine aromatische Diolkomponente umfaßt.

8. Empfangsblatt für den Thermotransferdruck nach Anspruch 7, worin die aromatische Diolkomponente in einem größeren molaren Anteil als die alicyclische Diolkomponente enthalten ist.

9. Empfangsblatt für den Thermotransferdruck nach Anspruch 8, worin die aromatische Komponente der Diolmischung ein Ethylenoxid- oder Propylenoxidadukt eines Bisphenols umfaßt.

10. Empfangsblatt für den Thermotransferdruck nach Anspruch 1, worin die alicyclische Diolkomponente des Polyesters ein Cyclohexangrundgerüst aufweist.

11. Empfangsblatt für den Thermotransferdruck nach einem der vorhergehenden Ansprüche, worin die farbstoffempfangende Schicht zusätzlich zum Copolyester und einem beliebigen, polymeren Ablösemittel, das eingesetzt werden kann, einin geringeren Anteil eines anderen polymeren Materials enthält, das intensiv mit dem Copolyester gemischt ist.

12. Empfangsblatt für den Thermotransferdruck nach einem der vorhergehenden Ansprüche, worin die polyesterartige Quervernetzung des Copolyesters durch Umsetzung mit einer wirksamen Menge eines dafür vorgesehen Quervernetzungsmittels verbessert wird.

13. Empfangsblatt für den Thermotransferdruck nach einem der vorhergehenden Ansprüche, in dem ein Antistatikmittel auf eine oder mehrere Beschichtungen des Empfangsblattes aufgetragen wird oder in eine oder mehrere Schichten des Empfangsblattes eingebracht wird.

14. Empfangsblatt für den Thermotransferdruck nach Anspruch 13, worin die Antistatikbehandlungen auf beiden Seiten des Trägers angewendet werden.

15. Thermotransferdrucksystem, umfassend ein Farbstoffblatt, das Thermotransferfarbstoffe enthält, und ein Empfangsblatt zum Empfang der Farbstoffe während des Thermotransferdruckens, worin das Empfangsblatt ein Empfangsblatt nach einem der Ansprüche 1 bis 14 ist.

## Revendications

1. Feuille réceptrice pour l'impression par transfert thermique comprenant un substrat dont une surface porte une couche réceptrice pour un colorant dans laquelle le principal composant de la couche réceptrice pour le colorant est un copolyester dans lequel le composant acide comprend au moins un acide dicarboxylique alicyclique et le composant alcool comprend au moins un diole alicyclique.

2. Feuille réceptrice pour l'impression par transfert thermique suivant la revendication 1, dans laquelle le composant acide du copolyester comprend un mélange d'un composant acide dicarboxylique alicyclique et d'un autre composant acide polycarboxylique ayant un rapport molaire compris dans la gamme de 5/95 à 95/5.

3. Feuille réceptrice pour l'impression par transfert thermique suivant la revendication 2, dans laquelle le composant acide du copolyester comprend un composant acide dicarboxylique alicyclique et un composant acide dicarboxylique aromatique.

4. Feuille réceptrice pour l'impression par transfert thermique suivant la revendication 3, dans laquelle le composant acide dicarboxylique aromatique est présent en une proportion molaire supérieure à celle du composant acide dicarboxylique alicyclique.

5. Feuille réceptrice pour l'impression par transfert thermique suivant la revendication 3 ou la revendication 4, dans laquelle le composant acide dibasique aromatique comprend au moins un composé parmi l'acide téréphtalique ou l'acide isophtalique.

6. Feuille réceptrice pour l'impression par transfert thermique suivant la revendication 1, dans laquelle le composant alcool du copolyester comprend un mélange d'un composant diol alicyclique et d'un autre composant alcool polyhydrique selon un rapport molaire compris dans la gamme de 5/95 à 95/5.

7. Feuille réceptrice pour l'impression par transfert thermique suivant la revendication 6, dans laquelle le composant alcool du copolyester comprend un composant diol alicyclique et un composant diol aromatique.

8. Feuille réceptrice pour l'impression par transfert thermique suivant la revendication 7, dans laquelle le composant diol aromatique est présent en une proportion molaire supérieure à celle du composant diol alicyclique.

9. Feuille réceptrice pour l'impression par transfert thermique suivant la revendication 8, dans laquelle le composant aromatique du mélange de diols comprend un produit d'addition d'oxyde d'éthylène ou d'oxyde de propylène d'un bisphénol.

10. Feuille réceptrice pour l'impression par transfert thermique suivant la revendication 1, dans laquelle le composant diol alicyclique du polyester a un squelette cyclohexane.

11. Feuille réceptrice pour l'impression par transfert thermique suivant l'une quelconque des revendications précédentes, dans laquelle en plus du copolyester et d'un quelconque agent de détachement polymère susceptible d'être employé, la couche réceptrice pour un colorant contient une quantité mineure d'autres matériaux polymères étroitement mélangés au copolyester.

12. Feuille réceptrice pour l'impression par transfert thermique suivant l'une quelconque des revendications précédentes, dans laquelle la réticulation du type polyester du copolyester est augmentée par réaction avec une quantité efficace d'un agent de réticulation pour celui-ci.

13. Feuille réceptrice pour l'impression par transfert thermique suivant l'une quelconque des revendications précédentes, dans laquelle un agent antistatique est déposé sur un ou plusieurs revêtements du récepteur ou incorporé à ceux-ci.

14. Feuille réceptrice pour l'impression par transfert thermique suivant la revendication 13, dans laquelle les traitements antistatiques sont appliqués sur les deux faces du substrat.

15. Système pour l'impression par transfert thermique comprenant une feuille de colorants contenant des colorants pour transfert thermique et une feuille réceptrice pour recevoir les colorants pendant l'impression par transfert thermique dans lequel cette feuille réceptrice est une feuille réceptrice suivant l'une quelconque des revendications 1 à 14.
